

2,967,104

## MAGNESIUM-BASE ALLOY

John F. Pashak, Linwood, Mich., assignor to The Dow Chemical Company, Midland, Mich., a corporation of Delaware

No Drawing. Filed June 5, 1957, Ser. No. 663,601

4 Claims. (Cl. 75—168)

The invention relates to magnesium-base alloys. It more particularly concerns magnesium-base alloys containing both thorium and manganese and having among other desirable properties high creep strength and rollability.

The desirable property of lightness in weight of magnesium is of little value in stressed parts because of its relatively low tensile strength especially at more or less elevated temperatures. Attempts to produce alloys having magnesium as a base that are light and not only possess high strength at more or less elevated temperatures but also are capable of being rolled readily into sheets and plates have met many difficulties. Among the magnesium-base alloys having good creep resistance is the ternary alloy of magnesium, thorium, and manganese disclosed in U.S. Patent 2,774,664. This alloy contains from 0.5 to 8 percent of thorium and from 0.2 to 2 percent of manganese. Although it is possible to roll this alloy into sheet and plate, this is difficult and wasteful of metal because the metal during rolling cracks at the edges entailing waste. The rolling difficulty is due in part at least to the low malleability of the alloy. According to the present invention, this difficulty is reduced if not entirely overcome by appropriate additions of zirconium.

The invention then is based upon the discovery that the magnesium-base magnesium-manganese-thorium ternary alloy tolerates the inclusion of small amounts of zirconium in spite of the presence of manganese which has been taught heretofore to prevent effective alloying of zirconium with magnesium-base alloys containing manganese. In this invention but a small amount of zirconium is required, an amount which is tolerable in spite of the presence of manganese.

0.2 to 2 percent of manganese are alloyed with magnesium and sufficient zirconium is added to more or less saturate the alloy while molten, this amount being from about 0.001 to 0.15 percent depending on the manganese content.

That is, at the lower end of the range of the manganese content larger amounts of zirconium can be tolerated, as up to 0.15 percent when the manganese content is 0.2 percent; and at the higher end of the range of manganese content, the smaller the amount of the zirconium that can be tolerated, as 0.001 percent zirconium when the manganese content is 2 percent. The preferred range of proportions of the alloying constituents are from 1.5 to 3.5 percent of thorium, 0.4 to 1.0 percent of manganese, and from 0.001 to 0.05 percent of zirconium, the balance being magnesium except for incidental impurities which may be present in the metals used. Usually the total amount of incidental impurities does not exceed 0.3 percent of the weight of the alloy. A specific alloy composition having general application within the scope of the invention is one composed of 2.0 percent of thorium, 0.6 percent of manganese, and 0.01 percent of zirconium, the balance being magnesium.

The order in which the metals are alloyed does not appear to be critical. It is generally preferable to first melt the magnesium required as in a steel pot with a suitable saline flux for magnesium, such as one composed of 50 parts of potassium chloride, 30 parts of barium chloride, 15 parts of magnesium chloride, 5 parts of calcium fluoride. Following the melting of the magnesium, the requisite amounts of the other metals are added. The melt is stirred for as long as 10 to 20 minutes to ensure solution of the alloying metals in the molten magnesium. After the alloying is completed as described, a suitable saline refining flux may be added such as one composed of 95 percent of barium chloride and 5 percent of calcium fluoride and the melt stirred. The fluxed melt so obtained, either with or without the use of the refining flux, is allowed to settle by holding it quiescent for a time, e.g. 20 minutes. The supernatant molten alloy is decanted or otherwise separated from the flux and removed from the pot as desired and cast in a suitable mold.

It is generally preferable in preparing the alloy for rolling to cast the metal into ingot before rolling into sheet. In the rolling reductions in thickness of up to 20 percent per pass may be made.

The following tabulation of alloys made in accordance with the foregoing method is illustrative of the invention. In the examples of Table I the specimens were rolled from cast ingot heated to about 900° F.

Table I

| No. <sup>2</sup> | Alloy                |            |            | Properties <sup>1</sup> |     |     |    |           |     |    |        |           |     |    |        |
|------------------|----------------------|------------|------------|-------------------------|-----|-----|----|-----------|-----|----|--------|-----------|-----|----|--------|
|                  | Composition, Bal. Mg |            |            | 70° F.                  |     |     |    | 400° F.   |     |    |        | 600° F.   |     |    |        |
|                  | Percent Th           | Percent Mn | Percent Zr | Percent E               | TYS | CYS | TS | Percent E | TYS | TS | .5% EX | Percent E | TYS | TS | .5% EX |
| 1-----           | 2.3                  | 0.6        | 0.01       | 7                       | 26  | 25  | 35 | 13        | 20  | 24 | 12     | 19        | 12  | 15 | 4.2    |
| 2-----           | 2.6                  | 0.5        | 0.04       | 7                       | 27  | 24  | 35 | 15        | 21  | 24 | 13     | 25        | 11  | 15 | 4      |
| 3-----           | 2.7                  | 0.44       | 0.05       | 9                       | 28  | 26  | 35 | 17        | 20  | 22 | 11     | 40        | 9   | 13 | 3.6    |
| 4-----           | 2.8                  | 0.18       | 0.15       | 10                      | 28  | 24  | 34 | 20        | 20  | 22 | 7.3    | 78        | 5   | 11 | 0.6    |
| 5-----           | 2.6                  | 0.09       | 0.49       | 7                       | 28  | 25  | 35 | 17        | 21  | 23 | -----  | 92        | 6   | 11 | 0.8    |

<sup>1</sup> Sheet rolled from cast ingot at 900° F. Stress in 1000's p.s.i. TYS, the tensile yield strength and CYS, the compression yield strength, were measured at 0.2% deviation from the modulus line.

<sup>2</sup> All specimens have equiaxed grain structure.

.5% EX: In this column is given the load in 1000's of p.s.i. at which the specimen exhibits a total extension of .5 percent in length in 100 hours.

In carrying out the invention in its broadest aspects from 0.5 to 8 percent by weight of thorium and from

The alloy may be extruded readily at suitably elevated temperature and exhibits desirable mechanical properties

especially increased ductility as shown in the comparative data in Table II of an alloy prepared in accordance with the invention and a related parent ternary alloy for comparison.

2. A magnesium-base alloy containing from 1.5 to 3.5 percent of thorium, 0.4 to 1.0 percent of manganese, and from 0.01 to 0.05 percent of zirconium, the balance being magnesium.

Table II

| Alloy      |             |            | Extrusion Conditions |            |                 |                   | Properties <sup>1</sup> |         |          |          |          |
|------------|-------------|------------|----------------------|------------|-----------------|-------------------|-------------------------|---------|----------|----------|----------|
| No.        | Composition |            | Grain Type           | Temp., °F. | Speed, ft./min. | Reduction in area | Percent E               | TSY     | CYS      | TS       |          |
|            | Percent Th  | Percent Mn |                      |            |                 |                   |                         |         |          |          |          |
| 6<br>Blank | 3.2<br>3.4  | 1.6<br>1.7 | 0.003                | E<br>C     | 800<br>800      | 5<br>5            | 90:1<br>90:1            | 10<br>1 | 40<br>38 | 32<br>30 | 44<br>44 |

E=equiaxed grain structure; C=columnar grain structure; TYS and CYS means tensile yield strength and compression yield strength, respectively, at 0.2% deviation from the modulus line.

<sup>1</sup> Stress in 1000's p.s.i.

Among the advantages of the invention are that the alloy resists work hardening so that a substantial amount of cold working is possible without excessive work hardening; the alloy resists surface and edge cracking during rolling so that large thickness reductions per pass are possible, thereby saving rolling time and avoiding waste of metal; the alloy resists tearing during extrusion as on die expressing objects, such as bars, tubing, angles, etc., as a result a desirable surface is exhibited on extruded shapes especially those produced at the low temperatures at which maximum mechanical properties are obtained.

I claim:

1. A magnesium-base alloy containing from 0.5 to 8 percent of thorium, 0.2 to 2.0 percent of manganese, and from 0.001 to 0.15 percent of zirconium, the balance being magnesium.

20 3. A magnesium-base alloy containing 2.0 percent of thorium, 0.6 percent of manganese, 0.01 percent of zirconium, the balance being magnesium.

25 4. A magnesium-base alloy consisting of 0.5% to 8.0% thorium, 0.2% to 1.0% manganese, 0.05% to 0.15% zirconium, the balance being magnesium.

#### References Cited in the file of this patent

##### UNITED STATES PATENTS

30 2,774,664 McDonald \_\_\_\_\_ Dec. 18, 1956  
2,788,272 Whitehead et al. \_\_\_\_\_ Apr. 9, 1957

##### FOREIGN PATENTS

35 511,137 Great Britain \_\_\_\_\_ Aug. 9, 1939  
591,225 Great Britain \_\_\_\_\_ Aug. 12, 1947